

## UNITED STATES PATENT OFFICE

2,317,205

## METHOD OF WORKING METALS

Rudolf Lowit, Auburn, Maine, assignor to Callite  
Tungsten Corporation, Union City, N. J., a cor-  
poration of Delaware

No Drawing. Application March 6, 1940,  
Serial No. 322,574

## 12 Claims. (Cl. 117—49)

This invention relates to novel methods of coating metal surfaces with a carbon layer incident to its working, as well as to novel methods for cleaning the surface particularly of molybdenum, tungsten or their respective alloys.

The present method of making tungsten and molybdenum ductile at room temperature was first developed in 1909, and the essential procedure has remained substantially the same to date. By this process, the metal, in powder form, is first pressed into a bar of square section, which is then subjected to presintering and sintering stages. The bar at this stage is solid but brittle. In the manufacture of wire the bar is then subjected to a mechanical hammering process termed swaging, which hammers the bar into a wire form of substantially reduced cross section, such as of the order of 1.5 millimeters diameter. The swaging operations are accompanied by heating, generally below the recrystallization temperature of the metal.

At the present time, the most extensive use of tungsten is in the form of fine wires for filaments of incandescent lamps and as cathode and heater elements in electronic tubes. Molybdenum wire is used for hooks, supports and grid electrodes of electronic tubes and for heating elements of electric furnaces. Such wires range in diameter from approximately 1.25 down to 0.03 millimeter. The wire is initially swaged or rolled, generally down to a diameter of about 1.5 millimeters. The final stage in forming the ductile fine wire consists in drawing it through suitable dies to reduce its diameter, in conjunction with suitable heating and annealing operation.

In drawing the wire, there is a drum on which the wire is wound, a graphite lubricant bath for coating the wire, a die, and a second drum driven by suitable motivating means for taking on the drawn wire. A heated zone is arranged about the wire, to suitably heat it prior to its passage through the die. The heating serves to bake the graphite coating onto the wire, and to soften the wire for facilitating its drawing to smaller diameters. The die itself is generally also heated. The ductility of the wire increases with continuous drawing and the wire may eventually be drawn cold in the smallest diameters. The speed of the drawing depends upon the wire diameter. The heat treatment during drawing is such that the wire temperature is kept below the recrystallization point of the metal to prevent embrittlement of the wire. Reduction in diameter upon each passage of the wire through the die generally ranges between 5 and 10 per cent.

It is important to have a protective coating on the wire to serve as a lubricant in the drawing to prevent abnormal die wear. This coating also protects the wire surface from oxidation during heating applied in the swaging as well as the drawing stages of these metals. The protective coating generally used is graphite. The coating has heretofore been applied on the rod, wire or ribbon in the final stage of the swaging and for all the drawing operations by passing it through a bath containing graphite in suspension or emulsion. Heating bakes the graphite coating on the wire. The graphite coating should preferably be homogeneous in nature for successful commercial results.

Heretofore it has been difficult to insure a homogeneous coating of this nature on rods or wires of tungsten and molybdenum. A non-homogeneous coating results in surface irregularities and abrasion of the drawn wire, as well as in appreciable wear on the die, producing wire with inferior physical properties. This was due to increased and irregular friction between the die and the wire, resulting in excessive strains in sections of the wire. Commercially, the resultant wires were rejected in substantial measure in their manufacture. The prior surface coating of such wire in their working stages generally comprised besides the graphite, metallic oxides, abraded metal, and other impurities incurred during the successive hot working stages. The resultant layer was non-uniform, and it was heretofore commercially impractical to affix homogeneous coatings in the successive stages.

Several methods were heretofore used to clean the surface of molybdenum and tungsten wire for coating or recoating with graphite during some stage in its working. The coating on such wire with a diameter greater than about one millimeter was in some cases removed by passing the wire through a fused bath of sodium nitrite. However, precaution had to be taken to keep the loss of the pure metal itself to a minimum. In another method tungsten wire was immersed for 30 minutes in boiling sodium or potassium hydroxide, then thoroughly washed with water and finally cleaned with felt pads. A further surface cleaning method was to raise the wire to incandescence in a reducing atmosphere. However, there were the dangers of undesirable effects upon the crystal structure of the metal and the formation of compounds on its surface.

In accordance with my present invention I provide improved methods for cleaning impurities from the surface of molybdenum, tungsten and

their alloys, and for uniformly coating such metals with a firmly adherent and homogeneous carbon layer to give substantially improved control in their metal working and uniform physical properties in the completed product. Broadly speaking, one phase of my invention comprises treating such metal with a chemical oxidizer to first loosen all its surface impurities. I have found that a solution containing potassium permanganate is most suitable as such oxidizer. It is to be understood, however, that other suitable oxidizers may instead be used. Upon loosening the surface coating with the oxidizer, the metal is then treated with a cleaning solvent which does not appreciably attack the pure metal itself. I have found hydrochloric acid very suitable for such cleaning. Heating is not required for this cleaning process, and therefore the crystal structure of the metal is not adversely affected.

A very important feature of my present invention is my novel method for coating a metal surface with a protective carbon layer, such as graphite. Two classes of metals may be so treated; firstly, those that are usually hot-worked or drawn such as tungsten, molybdenum or their alloys, and secondly, those metals which are usually cold-worked or drawn with difficulty. Where impurities have been deeply imbedded in the metal surface such as due to prior working, the metal is preferably first cleaned of its surface impurities in some suitable manner, for example as my my novel cleaning process previously described. Upon cleaning, the metal is introduced into an oxidizing solution to condition its surface for the subsequent coating of carbon or graphite which homogeneously adheres onto the conditioned surface. I found potassium permanganate solution very suitable as the conditioner for this purpose. When the thus conditioned metal has carbon or graphite applied to it, and is subsequently heated, an adherent layer thereof is baked thereon. When wire is coated in this manner, the carbon or graphite layer serves to protect its surface, and to lubricate the drawing action. Other uses for such graphite or carbon layers are indicated, such as in "black-body" electrodes for radio tubes.

I have found that in some cases it is unnecessary to clean or otherwise completely remove the surface impurities from the metal in its working, such as in swaging or wire drawing. The wire with its old or worn graphite coating is treated with the oxidizing or conditioning solution, whereupon the layer thereon is conditioned. When the thus treated wire is then passed through the graphite suspension a resultant homogeneous layer is produced by the new graphite combining with the conditioned old layer.

It is accordingly an object of my present invention to provide a novel method of cleaning surfaces of molybdenum, tungsten or their alloys.

Another object of my present invention is to provide novel methods of removing coatings of graphite and other impurities from molybdenum, tungsten or their alloys.

Still another object of my present invention is to provide novel methods of homogeneously coating metals with a carbon layer.

A further object of my present invention is to provide improved methods of continuously coating a wire with a graphite layer.

These and further objects of my present invention will become apparent in the following description of preferred methods for carrying out the invention.

In accordance with one aspect of my present invention, the surface of molybdenum, tungsten or their respective alloys is cleaned of surface impurities with a loosener or oxidizing agent that first loosens the impurities and a subsequent cleaner solution. Surface impurities encountered in working the metal generally comprises carbon such as graphite from the prior coatings, metallic oxides, abraded metal, and other impurities. The metal, in wire, rod, ribbon or sheet form, is first treated with a solution containing suitable oxidizer. In the case of molybdenum or its alloys with tungsten particularly where molybdenum predominates, I have found that solutions of the halates, perhalates, manganates and permanganates, etc., of the alkali and alkaline earth groups and also the acids of these anions and mixtures thereof are suitable oxidizers for this purpose. By the alkalies I refer to ammonium, sodium, potassium, etc. By the alkaline earths I refer to magnesium, calcium, barium, etc. By the halates I refer to chlorates, bromates and iodates, etc.; and by the perhalates to the perchlorates, perbromates and periodates, etc. In the case of tungsten, I have found that a suitable oxidizing solution is comprised of potassium permanganate together with a compound of the class including the oxides, peroxides, hydroxides, cyanides, carbonates, sulphites, sulphides, nitrates, nitrites of the alkali and alkaline earth group. The oxidizing loosener or solution is preferably heated to a temperature below its boiling point. The metal, when in wire form, may be linearly passed through the solution, or be arranged in a coil which is then placed therein for any desired period up to one hour or longer.

Treating the molybdenum or tungsten metal with oxidizing solution, loosens the usual graphite coating or adhering foreign particles from its surface. The metal may then be rinsed to remove loosened surface particles and excess oxidizing solution. Water may be used for this washing. The loosener or oxidizer undermines the cohesion of the surface impurities on the metal.

The remaining deposits on the metal surface may be completely removed by subjecting the treated metal to a cleaning solution. For molybdenum or its alloys with tungsten, I have found that a cleaning agent suitable for this purpose is amongst the group comprising hydrochloric acid, or a solution of halides of the alkali and alkaline earth groups; specifically chlorides, fluorides, bromides and iodides, and the acids of these anions or any combination of these. In the case of tungsten, a suitable cleaning agent is one of the class including hydrochloric acid, or oxides, peroxides, hydroxides, cyanides, carbonates, sulphites, sulphides, nitrates, nitrites of the alkali and alkaline earth groups. Such cleaning agent removes the residual coating and impurities on the metal surface without appreciably attaching or dissolving the metal itself. I prefer to use hydrochloric acid, and have found solutions 5 per cent by weight to the fully concentrated form satisfactory. Concentrated hydrochloric acid is very satisfactory commercially for this purpose for either molybdenum or tungsten or their alloys. It is to be noted that no evident loss of metal is en-

countered in the surface cleaning with my novel process, and that a wire thus cleaned remains uniform in diameter. Since the molybdenum, tungsten, or their alloys, are not appreciably attacked, the physical characteristics of wire thus cleaned remain intact, being controllable to insure a predetermined uniform diameter.

Heretofore cleaning molybdenum and tungsten was attempted in a single step with a relatively strong cleaning agent. However, the tenacious surface impurities encountered on such metals whether or not containing graphite were generally removed with difficulty by such single step cleaning due to the irregular character of the impurities. Such strong cleaning agents also appreciably attacked the metal surface in portions of least resistance before removing the more resistant impurities. With my two-step cleaning process herein the surface impurities are first converted or loosened on the metal and then treated with a cleaning agent which does not appreciably attack the metal itself, giving satisfactory and uniform results.

My invention further contemplates the coating of metal surfaces with graphite, or amorphous carbon in any other form. Such coating is particularly required in the hot drawing of wires and in some stages of hot rolling or swaging of molybdenum, tungsten and the respective alloys of these metals. The graphite coating impedes oxidation of the metal, and in hot drawing serves as a drawing lubricant, protecting the die from excessive wear and the wire from damage and undue strain. Metals which are usually cold-drawn with difficulty may be similarly treated to advantage. Such metals are those that have compounds formed on their surface which are hard, and difficult to remove, and which increase the die wear, as well as which impart inferior physical characteristics to the drawn wire. Stainless steel wire is an example of a metal of this class which is cold-drawn. Other metals in this class are some of the alloys containing chromium, molybdenum, tungsten, tantalum, cobalt or manganese. In the cold drawing process, the graphite coating does not serve as the lubricant, but rather acts primarily to protect the die and wire from the effects of the hard surface impurities. The lubricant used here is the one generally employed in cold drawing.

In accordance with my invention, the surface of the metal is cleaned of its impurities in any suitable manner. In the case of molybdenum, tungsten or their alloys, the surface impurities are advantageously removed by the hereinabove described two-step process employing an oxidizing solution and cleaning agent solvent. The clean metal surface is treated with a conditioning solution. Suitable conditioners for this purpose for the hot or cold worked metals are the loosener agents or oxidizers enumerated hereinabove for the surface cleaning processes of molybdenum, or tungsten, or their alloys. In the case of tungsten, I have found that a potassium permanganate solution alone also serves as a suitable conditioner when used on a cleaned tungsten surface. In commercial conditioning of molybdenum, tungsten or their respective alloys, I have found a solution containing potassium permanganate, for example between 0.3% to 3% of potassium permanganate by weight, very suitable for the surface conditioning. However, other concentrations thereof are feasible.

After partial or complete drying of the conditioned surface, it forms an excellent means for

securing graphite, carbon black, and the like onto the metal surface. I believe that the described conditioners, particularly potassium permanganate, form a deposit which is suspended among the carbon particles and facilitates the flow of the carbon particles during the metal working, particularly in wire drawing.

Where merely a carbon layer is desired on the metal, such as for use as an electrode element in an electronic tube, carbon black, or carbon in any other form is applied onto the conditioned surface, and preferably heated to firmly bake on the carbon layer.

Where the metal is to be cold-worked, particularly cold-drawn into wire, it is introduced to a graphite suspension subsequent to its conditioning as described. The graphite is then baked onto the conditioned wire surface and while hot the wire is preferably passed through a suitable drawing die which works the graphite into a firmly adherent layer thereon.

The usually hot-worked metals, namely of the class comprising tungsten, molybdenum or their respective alloys, are likewise coated with the protective layer of graphite or other suitable substance, by first conditioning the cleaned surface thereof with an oxidizer as described hereinabove, then preferably partially or completely drying the surface and then coating it with graphite. The heating accompanying the working, whether rolling, swaging or drawing, bakes the graphite layer firmly thereon. Where wire is formed by such methods, the conditioned wire is passed through the usual graphite suspension and the heating zone before reaching the rolling or swaging unit or die, and forms a tenacious and homogeneous protective coating thereon. The resultant wire is very uniform in physical properties. Due to this homogeneous protective graphite or other coating on the wire, no striations appear thereon, nor does undue tool or die wear take place. The resultant wire is produced with uniform ductility, diameter, tensile strength and elongation throughout its entire length, an important advantage in commercial production.

The metal surface cleaning and graphite coating processes of my present invention may be practised in various ways, for the different phases of the metal working or wire drawing. The coating of the metal with a protective lubricant layer, such as graphite, may for example be performed in a continuous manner in conjunction with the rolling, swaging or drawing operations. Wire containing an old or injured graphite coating is first passed through an oxidizing solution (such as for example the 0.3 to 3% solution of potassium permanganate by weight referred to above) to act on the old coating and to condition the surface. The wire is then passed through the usual graphite bath, or equivalent compound. The graphite suspension firmly attaches itself to the conditioned surface of the wire and admixes with the old coating thereon to form a resultant homogeneous graphite layer. In hot working, when the wire is next moved through the usual heating zone, all in a continuous process, the graphite suspension dries on its surface and is baked thereon as an adherent coating. For this continuous procedure the previous intermediate stage for wire cleaning per se is omitted. The graphite coated wire is then passed through the rolling or swaging unit or die in the usual manner, resulting in a uniform metal product. A coil of wire may be dipped as a whole into the

conditioner or oxidizing solution, and subsequently introduced linearly to the continuous process of graphite coating and hot working.

In my novel continuous procedure of recoating the metal wire, the passage of the wire through my oxidizing solution or conditioner prior to its passage through the graphite bath, is essentially what is additional to the prior art wire-working procedure. In the preferred case, the wire is introduced to or passed through a solution of potassium permanganate as the conditioner and then to the graphite bath.

Another important feature of my invention is concerned with its use in connection with annealing metals in any shape, such as in the form of wire, of the group consisting of tungsten, molybdenum, or their respective alloys. If such metals are annealed with foreign particles on their surfaces, there is great likelihood that the particles would react with the metal and impart undesirable physical properties to the product. I propose to treat the metal or wire to be annealed by the described conditioning treatment, such as with the potassium permanganate solution, to loosen these particles, and subsequently washing, and also scrubbing if desired, to remove the foreign particles. The resultant coating is preferably removed by a cleaning agent such as by hydrochloric acid described, prior to the annealing stage. I have found that all impurities on the surface of the metal are removed and otherwise rendered inert so that upon subsequent heating or annealing in a suitable atmosphere, no chemical action ensues which causes deleterious effects on the metallic surface.

Although I have described preferred modes for carrying out my invention, it is to be understood that it may be practised in different ways falling within the broader spirit and scope of the invention, and accordingly I do not intend to be limited except as set forth in the following claims.

I claim:

1. The process of coating a metal of the group consisting of molybdenum, tungsten, chromium, nickel, iron, cobalt, tantalum and manganese, and their alloys, with carbon which comprises treating the metal with a solution containing potassium permanganate and applying the carbon onto the treated surface.

2. The process of treating a wire of the class of metals consisting of molybdenum, tungsten, chromium, nickel, iron, cobalt, tantalum and manganese, and their alloys, which comprises cleaning the surface of the wire, subjecting said wire to a solution containing potassium permanganate, coating the wire with a graphite layer and heating the coated wire to bake the carbon thereon.

3. The method of coating a wire of the class consisting of molybdenum, tungsten, chromium, nickel, iron, cobalt, tantalum and manganese, and their alloys, which comprises treating the wire with a solution containing potassium permanganate, subjecting the treated wire to hydrochloric acid, further applying a solution containing potassium permanganate to the wire, then coating the wire with a carbon layer and heating the coated wire to bake the carbon thereon.

4. The method of continuously recoating a carbon coated wire of the group consisting of tungsten, molybdenum, chromium, nickel, iron, cobalt, tantalum and manganese, and their alloys, which comprises treating the wire with a solution of potassium permanganate whereby the previously

applied coating of carbon is loosened and then applying graphite thereon.

5. The method of continuously recoating a carbon coated wire of the class consisting of molybdenum, tungsten, chromium, nickel, iron, cobalt, tantalum and manganese, and their alloys, with a layer of graphite which comprises subjecting the wire to a solution of potassium permanganate and then applying another layer of the carbon thereon.

6. The method of coating a metal wire of the group consisting of molybdenum, tungsten, chromium, nickel, iron, cobalt, tantalum and manganese, and their alloys, with a layer of graphite which comprises treating the wire with a solution of an oxidizing agent whereby a coating is formed on said wire of the reaction products of said oxidizing agent and said metal and then applying the graphite onto said coated surface.

7. The method of coating a metal wire of the class of molybdenum, tungsten, chromium, nickel, iron, cobalt, tantalum and manganese, and their alloys, with a layer of graphite which comprises treating the wire with a solution of an oxidizing agent whereby is formed a coating of the reaction products of said oxidizing agent with said metal, applying a layer of graphite onto the treated surface and baking the graphite layer onto the wire surface thereby forming on said surface a firmly adherent layer of carbon and said reaction products.

8. The method of coating the surface of a metal body of the class consisting of molybdenum, tungsten, chromium, nickel, iron, cobalt, tantalum and manganese, and their alloys, with a layer of graphite which comprises treating the metal with a solution of an oxidizing agent whereby the oxidizing agent reacts with the metal forming a coating thereon onto which the carbon adheres substantially better than onto the bare metallic surface, and then applying the graphite onto the coated surface.

9. The method of coating the surface of a metal of the class consisting of molybdenum, tungsten, chromium, nickel, iron, cobalt, tantalum, and manganese, and their alloys, with a layer of graphite which comprises treating the metal with an oxidizing solution which loosens particles on the metal surface, applying to the treated metal a cleansing agent which does not appreciably react with the metal itself but removes the loosened particles therefrom, thereafter subjecting the metal to a solution of an oxidizing agent which reacts with the metal forming a coating thereon onto which the graphite adheres substantially better than onto the bare metallic surface and then applying the graphite onto the coated surface.

10. The method of continuously recoating a carbon coated wire of the class consisting of molybdenum, tungsten, chromium, nickel, iron, cobalt, tantalum and manganese, and their alloys, with a layer of graphite which comprises treating the wire with a solution of an oxidizing agent and then applying another layer of graphite thereon.

11. The method of coating the surface of a metal body of the class consisting of molybdenum, tungsten, chromium, nickel, iron, cobalt, tantalum and manganese, and their alloys, with a layer of graphite which comprises treating the metal with an oxidizing solution that forms a coating of the reaction products of said solution and said metal and then applying the carbon onto the treated surface and baking said graphite into a firmly adhering layer with said coating.

12. The method of treating a metal wire of the group consisting of molybdenum, tungsten, chromium, nickel, iron, cobalt, tantalum and manganese, and their alloys, with a layer of graphite which comprises cleaning the surface of the wire, subjecting the cleaned wire to a solution of an oxidizing agent which reacts with the metal and

forms a coating thereon onto which the carbon adheres substantially better than onto the bare metallic surface, applying a layer of the carbon onto the coated surface and baking the carbon layer thereon.

RUDOLF LOWIT.